

# UNITED STATES PATENT OFFICE.

GEORGE W. HERBEIN, OF SEATTLE, WASHINGTON.

## ARTIFICIAL FUEL.

No. 901,707.

Specification of Letters Patent.

Patented Oct. 20, 1908.

Application filed November 30, 1907. Serial No. 404,634.

*To all whom it may concern:*

Be it known that I, GEORGE W. HERBEIN, a citizen of the United States, residing at Seattle, in the county of King and State of Washington, have invented certain new and useful Improvements in Artificial Fuel, of which the following is a specification, reference being had therein to the accompanying drawings.

10 This invention relates to artificial fuel; and it has for its object the provision of a fuel comprising a relatively large proportion of hydrocarbon in conjunction with an absorbent therefor, and a binding agent whose 15 viscous quality affords an exceedingly efficient cohesion of the constituents of the fuel and renders the mass into condition to assume the compressed form in which it is best fitted for consumption.

20 The fuel comprises as its essential ingredients, a hydrocarbon, such as petroleum oil; a combustible absorbent; and a binder therefor consisting of saccharate of lime.

I desirably employ peat as an absorbent 25 and combustible vehicle for the fluid constituents of the fuel. Its combustible quality is well known, and as an absorbent for the oil, in the proportions hereinafter stated, its efficiency is sufficiently demonstrated.

30 Besides these important functions the addition of peat to the oil involves certain reactionary effects shown by the effervescence following their union and by the alteration in the character of the petroleum caused 35 by the pyroligneous acid contained in the peat and which possesses an affinity for the fatty particles of the oil. The said reaction destroys a portion of the disintegrating character of the oil and renders it more

40 subservient to the binding agent and allows of a larger proportion of such high grade combustible being used. However, other substances of an absorbent quality and having a combustible value may be used in the

45 place of peat, such as garbage, saw-dust, or paper-waste, and may be found to be more available under certain conditions. Saccharate of lime, as used in this composition, has an extremely tenacious character which

renders it of great value as a binder. By 50 the employment of such binding agent opportunity is provided to economically utilize carbonaceous and ligneous matters of various kinds such as the disintegrated wastes of coal mines, which have heretofore been 55 difficult to combine in practicable fuel. The extreme cohesive nature of the binding agent renders possible the inclusion of a large percentage of such foreign combustible substances.

With the specific ingredients mentioned 60 the following proportions would yield a very satisfactory fuel, would when compressed retain its molded condition, withstand the effects of handling and the disintegration 65 due from combustion: petroleum, twenty per cent.; peat, seventy-eight per cent.; and saccharate of lime, two per cent. The petroleum is first heated and the peat, or other absorbent, is added and thoroughly 70 mixed until an intimate combination results; the saccharate of lime in a dry and powdered form is then added and thoroughly incorporated in the mixture, water being used to afford a consistency to the mass. 75 The mixture while still heated is compressed into the form of briquets and by allowing the heat and pressure to continue desirably for a period of twenty minutes the combustive quality of the fuel is improved and 80 the briquet is rendered impenetrable to water and practically unbreakable.

Having described my invention, what I claim, is—

1. An artificial fuel formed from petroleum, peat, and saccharate of lime in dry powder form.

2. An artificial fuel formed from petroleum twenty per cent., peat seventy-eight per cent., and powdered saccharate of lime 90 two per cent.

In testimony whereof I affix my signature in presence of two witnesses.

GEORGE W. HERBEIN.

Witnesses:

HORACE BARNES,  
ROBERT B. GILLIES.